

June 18, 1968

G. R. SOMERVILLE

3,389,194

METHOD FOR MASS PRODUCING SMALL SPHERICAL PARTICLES

Filed June 20, 1966

2 Sheets-Sheet 1



George R. Somerville  
INVENTOR

BY  
Browning, Sennar, Hager  
& Eickhardt  
ATTORNEY

June 18, 1968

G. R. SOMERVILLE

3,389,194

## METHOD FOR MASS PRODUCING SMALL SPHERICAL PARTICLES

Filed June 20, 1966

2 Sheets-Sheet 2



Fig. 2

George R. Somerville  
INVENTOR.

BY  
Browning, Seine, Heger  
& Eckhardt  
ATTORNEY

1

3,389,194

**METHOD FOR MASS PRODUCING SMALL SPHERICAL PARTICLES**

George R. Somerville, San Antonio, Tex., assignor to Southwest Research Institute, San Antonio, Tex.

Filed June 20, 1966, Ser. No. 558,796

5 Claims. (Cl. 264—4)

**ABSTRACT OF THE DISCLOSURE**

A method for mass producing capsules wherein there are a pair of concentric tubes opening into a conduit and filler and film material are fed into the inner and outer tubes, respectively, so as to extrude concentric rods of such materials from the ends of the tubes. A stream of carrier fluid is forced through the conduit and about the tube ends at a speed greater than the rate of extrusion so as to cause said rods to elongate and break off into individual segments which form into fluid capsules of filler material within the film material. In a preferred practice, the temperature of the carrier fluid is reduced below the melting point of the film material to harden it while the capsules are suspended in the stream.

This invention relates generally to a method for manufacturing small spherical particles, and has special utility in the manufacture of such particles in the form of capsules in which a filler material is contained within a seamless film material. More particularly, this invention relates to improved techniques for producing such particles, and especially such capsules, on a mass production basis.

In accordance with one prior technique, capsules of the type described are mass produced by means of centrifugal action. Thus, as shown and described in my prior Patent No. 3,015,128, a liquid film material is supplied to the interior of a rotating drum so as to extend across the inner ends of a bank of orifices disposed about and extending through the outer wall of the drum. Globules of the filler material are then delivered to the film material across the orifices, and the speed of rotation of the drum is such that the resulting centrifugal force overcomes the adhesive forces of the film material at the orifices so that it forms a shell about each filler material globule and is severed and flung outwardly from the orifices. As each capsule is so severed, additional film material forms across the orifice to receive an additional filler material globule, and all the fluid capsules are hardened in a suitable manner, such as within a bath of liquid hardening medium located to receive the capsules as they are flung from the orifices of the encapsulating drum.

Although this represents a substantial advance in the encapsulating art, it nevertheless has certain shortcoming when the filler material and film material have appreciably different densities. Thus, in this event, the centrifuging effect has a tendency to displace the globule of filler material off-center with respect to the shell of liquid film material. This eccentricity may be aggravated when the fluid capsules are flung into a liquid hardening medium, because of the impact of the capsule with the medium or collision with another capsule.

In accordance with another prior technique, the filler and film materials are extruded in the form of concentric fluid rods, which are caused to break off into individual fluid capsules by gravity or by vibration. Although this method is not as sensitive to density differences between the filler and film materials as the centrifugal method, it is nevertheless a much slower process and thus not capable of as high a rate of production. Furthermore, when the fluid capsules are hardened in a liquid hardening medium, there is the additional problem, above mentioned,

2

of shifting the filler material off-center due to impact of the capsules with the medium as well as collision with one another. These latter problems increase as the extrusion rate is increased, because of the more severe impact of the fluid capsules with the fluid hardening medium.

A still further difficulty encountered with the use of a liquid hardening medium, in these or other methods of forming spherical particles in which successive particles are directed toward the same point in the hardening medium, is their tendency to agglomerate.

10 There is often a need, in different types of known encapsulating methods, for accurately controlling the temperature of the fluid capsule when the film material is a hot melt. Shells of the film material are frequently of low strength when in the fluid state, and the rate at which they are cooled is critical. Solidification at too rapid a rate may result in deformed capsules, whereas solidification at too low a rate may result in excessive capsule breakage.

15 An object of this invention is to provide a method for mass producing spherical particles, whether in solid or capsule form, which obviates one or more of the foregoing difficulties, while at the same time enabling a very high rate of production.

20 Another object is to provide a method for mass producing capsules having outer shells of substantially uniform thickness, even though the filler and film materials have substantially different densities.

25 A more particular object is to provide such a method in which the fluid capsules may be hardened in such a manner as to avoid distortion.

30 A further object is to provide a method for mass producing small spherical particles, whether in solid or capsule form, in such a manner as to reduce the likelihood of their agglomerating in a liquid hardening medium, but without sacrificing the rates at which they may be produced.

35 A still further object is to provide an encapsulating method in which the temperature of the shell of a hot melt may be conveniently controlled in a manner to prevent damage thereto.

40 These and other objects are accomplished, in accordance with the illustrative embodiments of this invention, by a method in which a rod of fluid material is extruded into a stream of carrier fluid which is chemically non-reactive and physically immiscible with such rod material and which is flowing at a speed greater than the rate of extrusion of the rod. More particularly, the speed of the carrier fluid is selected to cause the rod to elongate and break up into segments which form into individual spherical particles, which may then be hardened in a manner to be described. This stream of carrier fluid is also influential in separating the particles to minimize the possibility of collision prior to hardening. Still further, the size of the particles is inversely proportional to the speed of the carrier fluid, so that the latter may be regulated to form particles of different sizes.

45 In the mass production of particles in the form of capsules in which a filler material is encased within a seamless shell of film material, concentrically arranged fluid rods of the filler and film material are extruded into the stream of carrier fluid. As the film material breaks off from the rod, it quickly forms about the filler material which is broken off with it to form a fluid capsule, which is then conveyed by the stream of carrier fluid to a hardening area. Since this involves neither a centrifuging action nor any other action tending to move the filler material off-center, the resulting capsule will have a shell of uniform thickness.

50 55 60 65 70 75 80 85 90 95 In one embodiment of the invention, the shell of film material comprises a hot melt which is hardened while

suspended in the stream of carrier fluid. Thus, the carrier fluid is maintained at a temperature above the melting point of the film material as it flows past the extruded rod and then reduced below such point to harden the fluid capsules. As a result, the capsules are hardened before colliding with one another upon separation from the carrier fluid and collection. Also, of course, the heating of the carrier fluid permits the maintenance of a desired temperature gradient for the capsules.

In another embodiment, the shell is instead a material which is hardened by chemical reaction or by solvent extraction. In this case, the fluid capsules are introduced with the carrier fluid into a suitable liquid hardening medium. However, the carrier fluid in which the capsules are suspended will distribute them to random locations within the medium. Also, the stream of carrier fluid will agitate the medium to a certain extent, so as to further reduce the likelihood of the capsules colliding with one another before hardening in the medium. Still further, the carrier fluid is a liquid, such as water, collected in a vessel above the hardening medium contained therein, so that the fluid capsules settle gradually to random locations of the medium, thereby essentially eliminating impact.

The stream of carrier fluid is confined within a conduit connecting at its downstream end with the vessel for collecting the carrier fluid and separating the hardened capsules therefrom. The upstream end of the conduit is connected with a suitable means for pumping the carrier fluid therethrough at the desired speed. Preferably, the carrier fluid is recirculated from the vessel to the upstream end of the conduit by means of an auxiliary conduit connecting the vessel with the pumping means.

The concentric rods of fluid filler and film material are extruded from the ends of concentric tubes which extend into the conduit. Preferably, these tube ends are arranged concentrically within the conduit and face toward its downstream end.

In the drawings where there is shown, by way of illustration, one embodiment of the invention:

FIG. 1 is a diagrammatic view of apparatus constructed in accordance with the first-mentioned embodiment of this invention; and

FIG. 2 is a diagrammatic view of apparatus constructed in accordance with the second-mentioned embodiment of the invention.

With reference now to the details of the above-described drawings, the first-mentioned embodiment of the apparatus shown in FIG. 1 comprises a conduit 10 having an upstream section 10a of enlarged circular cross-section and a downstream section 10b of reduced circular cross-section and connected to the upstream section by means of a conical restriction 10c. Inner and outer concentric tubes 11 and 12 extend concentrically within enlarged conduit section 10a for extruding fluid rods of filler and film material into the conduit. As shown in FIG. 1, the open ends of the tubes 11 and 12 terminate substantially adjacent the conduit restriction 10c, while the opposite ends of the tubes extend through the closed end 13 of conduit section 10a for connection with reservoirs 14 and 15. Thus, film material may be contained within reservoir 14 for supplying it to the outer tube 12, and filler material may be contained within a reservoir 15 for supplying it to the inner tube 11. These materials are kept in a fluid state as they are forced from the reservoirs, through pipes 16 and 17 and into the tubes by means of metering pumps 18 and 18a, respectively.

Carrier fluid is forced into the upstream end of enlarged conduit section 10a so as to flow concentrically about the outer tube 12, and past the ends of the tubes, through the restriction 10, and into the reduced section 10b of the conduit. Obviously, as this carrier fluid flows through the restriction 10c, its velocity is increased, depending upon the relative sizes of the annular flowway within the section 10a and the flowway within section 10b. At any rate, in accordance with this invention, the

velocity is increased at this area adjacent the ends of the tubes 11 and 12 to a value sufficiently greater than the extrusion velocity of the film and filler materials through these tubes as to cause the concentric rods extruded therefrom to elongate and break off into segments which form into fluid capsules. As these capsules are broken off from the rod, they will flow suspended within the stream of carrier fluid through the reduced conduit section 10b.

As previously described, in this first embodiment of the invention, the film material which forms the shell of the capsule is a hot melt which is adapted to be hardened when cooled below its melting point. Thus, the stream of carrier fluid about the tubes is maintained at a temperature above the melting point of the film and filler material so that the fluid rods will remain liquid as they are extruded from the ends of the tubes and caused to break off and form into fluid capsules. These capsules then flow suspended within the stream of carrier fluid into and through the reduced conduit section 10b. As shown in FIG. 1, there is a counterflow heat exchanger 19 disposed about reduced section 10b for gradually decreasing the temperature of the carrier fluid from a point above the melting point of the film material to a point below such point. Thus, the suspended fluid capsules are caused to harden during their flow from the upstream to the downstream end of the reduced conduit section 10b. More particularly, the temperature gradient is in this way controlled during this time so as to avoid damage to the shell material, as might incur in the event the temperature of the film material was too rapidly or too slowly reduced.

Carrier fluid is supplied to the upstream end of enlarged conduit section 10a by means of an auxiliary conduit 20 connected at its upstream end with a source of carrier fluid, to be described hereinafter, and at its downstream end with the upstream end of the enlarged conduit section. This carrier fluid is moved through the auxiliary conduit and into the main conduit 10 at the desired speed by means of a pump 21 disposed within the auxiliary conduit upstream of a flowmeter 22 for indicating the flow rate of the carrier fluid. The temperature of this carrier fluid is raised to the desired level by means of a heat exchanger 23 in the auxiliary conduit between the flowmeter 22 and the upstream of reduced conduit section 10a.

The downstream end of reduced conduit section 10b is connected with a vessel 24 for collecting the carrier fluid and the capsules suspended therefrom. In this embodiment of the invention, it is contemplated that the carrier fluid will be a liquid, such as water, of higher specific gravity than the capsules. Thus, there is an outlet 25 from the vessel above the connection thereto of conduit section 10b, so that the hardened capsules rise to the upper level of the carrier fluid so as to spill with it over the edge of outlet 25 onto a screen conveyor 26. The hardened capsules will move on the conveyor from left to right so as to spill into a collection container 27, and a brush 28 is mounted beneath the right-hand end of the screen 26 for wiping capsules from the screen which tend to stick to it.

As previously described, the carrier fluid is preferably recirculated from the vessel 24 to the upstream end of the main conduit 10. For this purpose a container 29 is mounted beneath the left-hand end of the screen 26 to receive the carrier fluid which passes through it. Additional carrier fluid for make-up purposes may be introduced into the container 29 through a line 30 connecting therewith. The lower end of carrier fluid container 29 is connected with the upstream end of auxiliary conduit 20, so that carrier fluid may be recirculated into the main conduit 10. This recirculation of the carrier fluid has several advantages, particularly when it is of relatively expendable material, its recirculation permits the retention of some of its heat used in maintaining the film ma-

terial in a fluid state within at least a portion of conduit 10.

One or both of the tubes 11 and 12 may be adjusted longitudinally of the conduit 10, as well as with respect to one another in any conventional manner. In being adjustable relative to the conduit 10, the open ends of such tubes may be moved toward or away from the restriction 10c for adjusting the velocity at which the stream of carrier fluid moves about the extruded rods. The adjustment of the ends of the tubes relative to one another may be desirable in order to accomplish certain extrusion characteristics.

As previously described, the carrier fluid is chemically nonreactive and physically immiscible with the film material which forms the shell of the capsule. At the same time, the film material is a hot melt which may be hardened in response to the lowering of the temperature of the carrier fluid from a point above to a point below its melting point. Still further, the filler material is a substance which may be maintained in its fluid state at a temperature at which the film material is also maintained in its fluid state. Obviously, however, the filler material may or may not be hardened after extrusion. As an example of materials meeting these qualifications, the film material may comprise a molten wax, the carrier fluid may be water, and the filler material may also be water. These substances were formed into capsules approximately 1,000 microns in diameter and containing approximately 57% by water with apparatus having the following structural and operational characteristics:

#### STRUCTURAL CHARACTERISTICS

|                          | Inches                  |
|--------------------------|-------------------------|
| Enlarged conduit section | 0.580 I.D.              |
| Reduced conduit section  | 0.315 I.D.              |
| Outer tube               | 0.1875 O.D., 0.150 I.D. |
| Inner tube               | 0.050 O.D., 0.030 I.D.  |

Outer ends of the inner and outer tubes flush with one another and located 1½" upstream of the conical restriction.

#### OPERATIONAL CHARACTERISTICS

|                                     |          |       |
|-------------------------------------|----------|-------|
| Upper carrier fluid temperature     | ° C.     | 80    |
| Lower carrier fluid temperature     | ° C.     | 50    |
| Filler material extrusion rate      | cc./min. | 30    |
| Encapsulating medium extrusion rate | cc./min. | 30    |
| Carrier fluid rate                  | g.p.m.   | 1 1/4 |
| Filler material temperature         | ° C.     | 80    |
| Encapsulating medium temperature    | ° C.     | 80    |

The same film, filler and carrier fluid materials were used in forming capsules approximately 1500 microns in diameter and containing approximately 57% water employing the same apparatus and the following operational characteristics:

|                                     |          |    |
|-------------------------------------|----------|----|
| Upper carrier fluid temperature     | ° C.     | 80 |
| Lower carrier fluid temperature     | ° C.     | 45 |
| Filler material extrusion rate      | cc./min. | 60 |
| Encapsulating medium extrusion rate | cc./min. | 60 |
| Carrier fluid rate                  | g.p.m.   | 2  |
| Filler material temperature         | ° C.     | 85 |
| Encapsulating medium temperature    | ° C.     | 85 |

The other embodiment of the apparatus shown in FIG. 2 is similar, in many respects, to the apparatus above-described in connection with FIG. 1. Thus, it includes a conduit 10' having enlarged and reduced cylindrical sections 10a' and 10b' connected by a restricted portion 10c', and concentric tubes 11' and 12' extending concentrically within enlarged conduit section 10a'. As in the first-described apparatus, filler material is fed in a liquid state to inner tube 11' and film material is fed in a liquid state to outer tube 12' from supply reservoirs 15' and 14', respectively, through pipes 17' and 16' having pumps 18' and 18a' respectively, disposed therein. Also, carrier fluid is introduced into the upstream end of enlarged conduit

section 10a' at the desired speed through an auxiliary conduit 20' connected at its opposite end to a source of supply of carrier fluid. As in the first embodiment of the invention, such carrier fluid is forced through the auxiliary conduit by means of a pump 21', and the flow rate thereof is measured by means of a meter 22'.

However, as previously mentioned, in this second embodiment of the invention, the fluid capsules broken off from the fluid rods extruded through the tubes 11' and 12' are hardened either by chemical reaction or solvent extraction, so there is normally no need for heat exchangers either in the restricted conduit section 10b' or in the auxiliary conduit 20'. Thus, in this second embodiment, the suspended fluid capsules flow entirely through the restricted conduit 10b' in a fluid state and into a vessel 31 adapted to contain a liquid hardening medium as well as to collect the carrier fluid and capsules.

In the illustrated embodiment of FIG. 2, it is contemplated that the carrier fluid will be a liquid having a lower specific gravity than the liquid hardening medium, and that the fluid capsules will have a specific gravity intermediate that of the fluid carrier and the hardening medium. Furthermore, the liquid carrier fluid and the hardening medium are also immiscible with one another so that they will stratify in the vessel 31 to establish an interface 33. The end of the restricted conduit section 10b' turns down to a level within the vessel below the upper level 32 of the carrier fluid, but above the interface 33 between the carrier fluid and hardening medium. As a result, the liquid capsules will gradually fall through the carrier fluid to the interface level 33. Also, this introduction of carrier fluid into the vessel 31 will agitate the fluid within the vessel so as to normally distribute the fluid capsules thereabout, and thus reduce the possibility of collision with one another prior to hardening at the interface level 33.

The interface level 33 is maintained by level control 34 at the upper open end 35a of overflow tube 35. The lower end of tube 35 is disposed above a screen conveyor 36 similar to the screen conveyor 26 shown in FIG. 1. Thus, the hardened fluid capsules and hardening medium spill over the open upper end 35a of the tube onto the screen 36, where, as described in connection with the apparatus of FIG. 1, the capsules are moved by the conveyor from left to right so as to spill into a container 37 disposed beneath the right-hand end of the conveyor. Also, blade 38 is used to wipe capsules from the conveyor in the event they have a tendency to stick to it.

The liquid hardening medium which spills over into the tube 35 and through the screen 36 is collected within another container 39 having its lower end connected by a pipe 40 to a pump 41, which recirculates it through a pipe 42 into the lower end of the vessel 31 beneath the interface 33. In the event there is a loss of hardening medium, as a result of which interface level 33 drops below the upper end of tube 35, the level control 34 will, through suitable means indicated by broken lines in FIG. 2, open a valve 43 within a make-up line 44 for admitting additional liquid hardening medium into the pipe 40 and thus into the lower end of the vessel 31. When the interface level has thus been brought back up to the desired level, the level control 34 shuts the valve in the make-up line.

The upstream end of auxiliary conduit 20' is connected to the vessel 31 above the interface 33, but below the upper level 32 of the carrier fluid, so that carrier fluid will flow into the conduit 20' and thus to the pump 21' and through flow meter 22' for recirculation into the upstream end of the main conduit 10'. There may be need for a scrubber 45 in the auxiliary conduit in order to assure that there is no premature hardening of the film material within the main conduit 10'.

As an example, this second embodiment of the invention may be used in the mass production of capsules comprising a filler material of hexane enclosed within a shell of aqueous sodium alginate. In this case, the carrier fluid

may be naptha, and the hardening medium may be aqueous calcium chloride, which converts the sodium alginate to insoluble calcium alginate. In this event, the carrier fluid might be scrubbed by liquid-liquid contact with water in the scrubber 45.

This invention has been illustrated and described in connection with the mass production of seamless capsules, because, as previously noted, it is especially well suited to such use. However, as also previously described, it also has utility in the mass production of solid spherical particles, and the term "particles," as used in the claims, contemplates either solid particles or particles in capsule form. As an example, it is contemplated that with suitable modification of the extruding means, this apparatus could be used in producing solid particles of wax. In this case, the carrier fluid could be water, which is immiscible with the wax and which may be maintained at a temperature level above the melting point of the wax as it flows past the extruding means and then lowered to a temperature level beneath the melting point of the wax after the fluid rod of the wax is elongated and broken off by means of the stream of carrier fluid into segments which form into spherical fluid particles.

From the foregoing, it will be seen that this invention is one well adapted to attain all of the ends and objects hereinabove set forth, together with other advantages which are obvious and which are inherent to the apparatus.

It will be understood that certain features and sub-combinations are of utility and may be employed without reference to other features and subcombinations. This is contemplated by and is within the scope of the claims.

As many possible embodiments may be made of the invention without departing from the scope thereof, it is to be understood that all matter herein set forth or shown in the accompanying drawings is to be interpreted as illustrative and not in a limiting sense.

The invention having been described, what is claimed is:

1. In a method of mass producing small spherical particles, the steps of extruding a rod of fluid material within a confined stream of carrier fluid which is chemically nonreactive and physically immiscible with said material and which is flowing at a speed greater than the rate of extrusion of said rod and moving in the same direction as said rod so as to cause said rod to elongate and break off into segments which form into individual fluid particles, maintaining the carrier fluid at a temperature above the melting point of the extruded rod as said carrier fluid flows therewith, and then reducing the temperature of the carrier fluid below such melting point to cool and harden the fluid particles while suspended in said stream of car-

rier fluid and thereby produce said small spherical particles.

2. In a method of mass producing small spherical particles, the steps of extruding a rod of fluid material within

5 a confined stream of carrier fluid which is chemically nonreactive and physically immiscible with said material and which is flowing at a speed greater than the rate of extrusion of said rod and moving in the same direction as said rod so as to cause said rod to elongate and break off into segments which form into individual fluid particles, and introducing the carrier fluid and the fluid particles suspended therein into a liquid hardening medium so as to harden the fluid particles within said hardening medium and thereby produce said small spherical particles.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999

ROBERT F. WHITE, Primary Examiner.

50 R. B. MOFFIT, J. R. HALL, Assistant Examiners.

#### References Cited

##### UNITED STATES PATENTS

2,265,801 12/1941 Cooke ----- 264—11

2,874,473 3/1959 Mitchell ----- 264—14

2,043,970 7/1962 Terenzi ----- 264—14 X

UNITED STATES PATENT OFFICE  
CERTIFICATE OF CORRECTION

Patent No. 3,389,194

June 18, 1968

George R. Somerville

It is certified that error appears in the above identified patent and that said Letters Patent are hereby corrected as shown below:

Column 8, line 47, "2,043,970" should read -- 3,042,970 --; same column 8 after line 47, insert the following references:

|           |         |        |         |
|-----------|---------|--------|---------|
| 3,092,553 | 6/1963  | Fisher | 264-14X |
| 3,111,708 | 11/1963 | Watt   | 264-4   |

Signed and sealed this 10th day of March 1970.

(SEAL)

Attest:

Edward M. Fletcher, Jr.

Attesting Officer

WILLIAM E. SCHUYLER, JR.

Commissioner of Patents